

(No Model.)

2 Sheets—Sheet 1.

F. RANSOME.  
MANUFACTURING CEMENT, &c.

No. 340,357.

Patented Apr. 20, 1886.



WITNESSES

J. L. Ouraud  
A. A. Smith

INVENTOR

Frederick Ransome  
By T. H. Robertson  
Attorney

(No Model.)

2 Sheets—Sheet 2.

F. RANSOME.  
MANUFACTURING CEMENT, &c.

No. 340,357.

Patented Apr. 20, 1886.



WITNESSES

J. L. Ourand.  
A. A. Smith.

INVENTOR

Frederick Ransome  
By T. J. W. Robertson  
Attorney

# UNITED STATES PATENT OFFICE.

FREDERICK RANSOME, OF LOWER NORWOOD, COUNTY OF SURREY,  
ENGLAND.

## MANUFACTURING CEMENT, &c.

SPECIFICATION forming part of Letters Patent No. 340,357, dated April 20, 1886.

Application filed January 18, 1886. Serial No. 188,942. (No model.) Patented in England May 2, 1885, No. 5,442.

*To all whom it may concern:*

Be it known that I, FREDERICK RANSOME, a subject of the Queen of Great Britain, residing at Lower Norwood, in the county of 5 Surrey, England, have invented certain new and useful Improvements in Manufacturing Cements, &c., (for which I have obtained an English patent dated May 2, 1885, and numbered 5,442,) of which the following is a 10 specification, reference being had therein to the accompanying drawings, in which—

Figure 1 represents a vertical longitudinal section; Fig. 2, an end view of the same, and Fig. 3 a cross-section through the line *y y*.  
15 This invention relates to a new process and apparatus for the manufacture of limes, cements, and similar substances.

The ordinary way of burning lime, cement, &c., is to place the materials in a kiln in blocks 20 or lumps, together with the fuel, and the two are thus burned together. It has also been proposed to effect the burning by feeding the material in a pulverized state into a rotating cylinder heated by a furnace arranged in close 25 proximity to one end of said cylinder where the fuel was burning, and the flames produced by the combustion entered directly into one end of the cylinder. This, although an improvement on the old plan, is wasteful of the 30 fuel, and is objectionable otherwise, owing to the ashes, sparks, and partly-consumed fuel, which are liable to mix with the cement.

According to my invention I use a (preferably) rotary cylinder heated by gas from a separate producer, which gas passes into the cylinder, together with sufficient air or steam, or both, to cause the combustion of the same, and thus produce an intense heat directly within the cylinder and among the particles of cement materials as the latter pass through the furnace, by which means not only are the materials more rapidly converted into cement, but all sparks, ashes, &c., are kept from mixing with the same. I also preferably feed the 40 material into the cylinder by means of a mechanical feeding device, by which it is fed into the cylinder in a regulated speed, whereby a greater uniformity of the quality of the material is obtained.

50 Referring now to the drawings by letter, A represents an inclined cylinder resting on roll-

ers B, running in suitable supports, C, mounted on the brick-work setting of the furnace, whereby the cylinder can revolve freely, like other revolving furnaces. Beneath the furnace is a shaft, D, supported on hollow blocks E, provided with fast and loose pulleys F, and a screw, G, which meshes into a ring of teeth, H, surrounding the cylinder, by which a slow revolving motion is given to the cylinder.

At H is a hopper, which is preferably provided with a suitable feeding device, as I, to which motion is imparted by a shaft, J, provided with a cone of pulleys, K, whereby the speed of the feeder may be regulated at will. Below this hopper and feeder is a curved pipe, L, the lower end of which terminates within the upper end of the cylinder. At the opposite or lower end of the cylinder there is a horizontal gas-pipe, M, which communicates by means of a pipe, N, with a gas-producer, O, which may be of any appropriate kind; but I prefer the form shown in the drawings. Between the pipe N and the horizontal pipe M is a valve, P, by which the amount of gas passing to the furnace is regulated. As shown, the pipe N, leading from the gas-producer O to the revolving furnace, descends to a trap, N', where any ashes, sparks, &c., that may pass off with the gas will be arrested and separated, so that nothing but gas passes to the furnace.

In the pipe M another pipe, R, is centrally secured, which pipe is provided at its outer end with a steam-nozzle, r, by which a jet of steam may be admitted, and thus a blast of air carried into the furnace with the gas. I sometimes provide the pipe R with means for partially or wholly closing its inlet, so that steam alone or more or less air may be admitted without especial regard to the amount of steam used.

Beneath the lower end of the cylinder A is a pit, Q, to which access may be had by an opening in the side. At the opposite end of the cylinder is a settling-pit, Q', arranged near the outlet to the chimney S, which latter is provided with a damper, T, for regulating its draft.

The cylinder is preferably made of boiler-iron of a suitable thickness, and lined with fire-bricks U u, those marked u projecting

further toward the center of the cylinder, for purpose that will hereinafter be explained.

The manner of using the above apparatus or making cement is as follows: Supposing the gas-producer to be charged with fuel and in operation and the steam-nozzle connected with a suitable supply of steam, the materials of which the cement is to be composed—such as clay and chalk—are first intimately mixed together, either in the dry or wet state. If in the wet state, the mixed materials or "slurry" is dried, then pulverized, and afterward sifted to bring it to the degree of fineness required in the cement. The finely-powdered material is then put into the hopper H, and the feeder I being moved at the regulated speed gradually and regularly feeds the material into the cylinder, which as it rotates keeps constantly turning the material over and over, so that every portion of the cement-making material is brought directly under the action of the intense heat within the cylinder, caused by the combustion of the gas from the gas-producer, and thus every particle of the cement so made has been subjected to the same degree of heat. The oxygen to support combustion is supplied through the pipe R, and is forced into the furnace in sufficient quantity by means of the steam-nozzle r. The turning of the material is much facilitated by the bricks u extending into the furnace, for they carry the material nearly up to the top of the upper side of the cylinder, from whence it falls in a stream down to the bottom side of the cylinder, passing through the intensely-heated and burning gases as it falls, when it again carried up and again falls through the burning gases. This is repeated again and again until the material has become thoroughly burned into cement and drops from the lower end of the cylinder into the pit Q, from which it is removed through the opening at e side.

It is obvious that limes or cements made with other materials than clay and chalk may be similarly reduced to powder of the requisite fineness before burning, and be then burned in the manner above described.

I regard the admixture of the gases from the producer with the requisite amount of oxygen in the revolving cylinder and the composition of the same therein as one of the essential features of my process, because by this mode of operation there is no liability of the fixture with the cement of objectionable matter, and the operation is more sure, thus producing a cement of uniform good quality, and especially is this the case when the trap

N' is employed. I also consider the regulation of the feed of the material into the cylinder as an important feature, as that also aids in procuring a uniform product.

In some cases I may place a grinding apparatus above the hopper and feeder, or use it as a substitute for the same, whereby one handling of the material is saved.

I do not claim, broadly, the making of cement by first grinding the material to a fine powder and then calcining the same, but

What I do claim as new is—

1. The process herein described of manufacturing cements, &c., which consists in first reducing the cement material to a powder and then burning the same in a suitable furnace by keeping it in a continuous movement there- 75 in while exposed to the flame produced by introducing into said furnace gas produced in a separate chamber distinct from the furnace, and mixing with said gas after it has left the gas-producer a suitable amount of oxygen, substantially as described.

2. The process herein described of manufacturing cements, &c., which consists in first reducing the cement material to a powder and then burning the same in a revolving chamber 80 while exposed to the flame produced by introducing into said chamber gas made in a separate producer distinct from the furnace, and mixing with said gas after it has left the gas-producer a suitable amount of oxygen, substantially as described.

3. The combination, in a cement-burning apparatus, of a revolving cylinder, a gas producer, and a trap between said gas producer and cylinder, substantially as described.

4. The combination, in a cement-burning apparatus, of a revolving cylinder, a gas producer, and a mechanical feeder, substantially as described.

5. The combination, in a cement-burning apparatus, of a revolving cylinder, a gas-producer, and a gas-pipe connecting said producer with the revolving cylinder, and an air-tube passing through said gas-pipe to supply the same with oxygen, whereby the air is heated by the gas and the two are mixed in the revolving cylinder, substantially as described.

In testimony whereof I affix my signature, in presence of two witnesses, this 4th day of January, 1886.

FREDERICK RANSOME.

Witnesses:

HERBERT E. DALE,  
W. JAMES S. KERTEN,  
Both of No. 17 Gracechurch Street, London.